

# UNITED STATES PATENT OFFICE.

CHARLES M. JOHNSON, OF AVALON, PENNSYLVANIA.

## PROCESS OF PRODUCING ALLOY STEELS.

1,366,662.

Specification of Letters Patent. Patented Jan. 25, 1921.

No Drawing.

Application filed December 12, 1919. Serial No. 344,329.

To all whom it may concern:

Be it known that I, CHARLES M. JOHNSON, residing at Avalon, in the county of Allegheny and State of Pennsylvania, a citizen 5 of the United States, have invented or discovered certain new and useful Improvements in Processes of Producing Alloy Steels, of which improvements the following is a specification.

10 My invention proceeds from the discovery that alloy steels may be produced in uninterrupted operation, beginning with iron oxid in the form of ore or scale; the smelting operation is accomplished in the presence 15 of both ferro-silicon and ferro-chromium, and such other non-ferrous metals as may be desired in the ultimate alloy are added in the form either of oxids; or of ferro-alloys, or of both. While not so specifically limited, my invention finds practical application to the production of high-speed steel, and I shall describe it in that 20 particular application; its applicability, however, to a wider field will be understood, 25 and in certain of the claims I shall define it in its wider scope and aspect.

In the narrower field of high-speed steel I have practised my invention with notable advantage in the following particulars: 30 First of all, reduction of such refractory material as high-speed scale, carried out in the presence of both ferro-silicon and ferro-chromium, becomes a much simpler operation; the smelting operation proceeds at a 35 much lower temperature than otherwise would be possible, and with consequent gain in the matters of fuel consumption and of wear and tear upon the furnace. High-speed scale is the scale which comes from the fabrication of articles of high-speed steel. It is an undesired by-product. Though rich in the valuable metals alloyed with the steel-tungsten, for example, commonly present in amounts as great as 11 or 40 12%, and vanadium in smaller amounts (about .4%),—it still has heretofore been so difficult of and so expensive of reduction, that in the eye of the steel maker it is of little value, and little better than a waste product. These difficulties I overcome, and 45 50 with manifest gain.

A second advantage lies in this; that, in

consequence of the lower temperature conditions prevailing during the smelting operation, the carbon component of the furnace charge (and, accordingly, of the finished product) may be kept low and kept under control, and, at the same time, when operating upon high-speed scale, all or substantially all of the more valuable alloying metals present—vanadium, tungsten, 55 chromium, etc., may be conserved. And, resulting from this, it follows that high-speed steel may be produced in uninterrupted operation, beginning with high-speed scale, or 60 other raw material. This is a procedure not heretofore attained, and commonly thought to be unattainable. The usual way is to begin with a derived material of relatively 65 low grade, ordinarily in high-speed steel 70 work a low grade ferro-tungsten containing vanadium. This derived material is the only product which heretofore has been derived from high-speed scale by direct operation. It is called "melting bar", although it is 75 not always in bar form. It is with this intermediate material that the production of high-speed steel, as such, ordinarily begins and, beginning with it, processes of refining 80 and of building up the desired alloy proceed. As I have now made abundantly plain, my invention begins, not with the intermediate product, but with the raw material out of which that intermediate product has previously been derived, that is to say, 85 with iron oxid (which may be high-speed scale), and proceeds thence in uninterrupted operation to the ultimate product, high-speed steel.

A third advantage of the application of 90 my invention to high-speed steel production lies in the incidental discovery of a steel of new composition, having individual characteristics, relatively inexpensive, but in performance excelling the most expensive high-speed steels of the present day. This steel 95 of new composition, hereinafter disclosed, I make the subject of an independent application for Letters Patent, Serial No. 344,320, filed December 12, 1919.

The results which I have attained are consequent upon a long series of experiments, to the ordering of which has gone much thought, and in the course of which advan-

55

60

65

70

75

80

85

90

95

100

tage has been taken of discoveries, both direct and incidental.

I can best describe my invention by rehearsing my actual operation, conducted on a scale which imparts to them an experimental aspect, although they are in constant and continuing use for commercial purposes. It will be understood that the actual performance is here given as a typical example, showing how my invention may be applied; latitude is permissible; this operation need not be slavishly followed. I shall, in the ensuing claims, define what is essential; and, so long as those essential things be adhered to, my invention will be practised, even though there be variation in other respects.

My initial furnace charge, of the actual operation alluded to, is—

High-speed scale, 300 pounds,  
20 Ferro-chromium, 20 pounds,  
Ferro-silicon, 27 pounds,  
Charcoal, 46 pounds,  
Molybdenum,  $2\frac{1}{2}$  pounds, and  
Tungsten,  $4\frac{1}{2}$  pounds.

25 The ferro-chromium and ferro-silicon are broken up and mixed together, and then mixed with the scale which constitutes the body of the furnace charge. The molybdenum and tungsten additions are made, 30 and their quantities are determined, according as the scale is rich or poor in these ingredients and capable or incapable of affording all that is needed in the finished product. The molybdenum which I introduce is of 78% purity and is in the form of powder; the tungsten also is in powdered form and is of 82% purity. These alloying metals are introduced (if at all) in the initial charge, rather than in subsequent additions, because (and this is peculiarly true of the tungsten), when so introduced, they do not in any appreciable degree enter into the slag, as is their tendency to do, if subsequently added.

45 The furnace charge so constituted, is brought to smelting temperature and the desired reactions ensue; the operation in this respect is the usual one, and further description is unnecessary.

50 Incidental to or, more properly speaking, consequent upon the smelting reactions, I find opportunity to bring the carbon component to the desired value. It is in anticipation of this that I keep the carbon constituent of the initial charge low (lower than sufficient to afford to the finished product its desired carbon content). When the smelting reactions have taken place, I sample the metal of the molten bath; allowing 55 the samples to grow cold, I subject them to fracture test, and judge thereby, whether the carbon content be proper. If it be too low, (as I intend and prefer it shall be) I build up the carbon content by charging in coke and stirring it into the bath. Under this

procedure the bath begins to carbonize at moderate speed, and, making tests at intervals of 10 or 15 minutes, I proceed until by fracture test I find the carbon content to have increased to the desired value. 70 Specifically, I get best results when I so proportion the initial charge that, when testing begins, the carbon content is in value .08 to .20% and I proceed with the addition of coke until the value rises to about .50%. It is best to begin with carbon low and then to build it up, because in so adding coke I incidentally restore to the bath the vanadium which initially has entered the slag. In case I find on the first test that the 80 carbon content is high—as high as or higher, let us say, than is ultimately preferable—.60% or more, I do not on that account abandon the furnace charge; I charge in more scale, rather, until I have reduced the 85 carbon to the preferred minimum of the normal operation (approximately .08%), and thence I proceed with the building up of the carbon, in the manner already described.

Having so brought the carbon component 90 of the bath to the desired value, it remains only to make certain final additions (not always made, however, as I shall presently explain), to bring the silicon, manganese and vanadium components to the desired 95 values. These, in the actual operation I am describing, are—

Ferro-silicon, 3 pounds,  
Ferro-manganese, 2 pounds, and  
Ferro-vanadium,  $5\frac{1}{2}$  pounds.

Tapping ensues.

I said a moment ago that final additions such as those just enumerated will not always be made. If, because of the composition of the scale used, the desired composition of the ultimate product may be had without these final additions, then of course, these will not be made. To be specific, in the case under consideration, if there be no final additions, the chromium content of the 110 finished product will range from a few tenths of one per cent. to 5% tungsten, from 12 to 13%; and vanadium, from .30 to 40%; and this may conceivably meet the specifications in hand.

115 Returning however to consideration of the operation as I normally and preferably conduct it, it remains to define the composition of the finished product, so far as concerns the elements which give it character as a 120 high-speed steel. This is—

Carbon, .67%,  
Manganese, .44%,  
Silicon, .63%,  
Chromium, 4.77%,  
Vanadium, 1.20%,  
Tungsten, 15.30%,  
Molybdenum, .60%.

125 Again I repeat, the figures are given with an accuracy exceeding necessity, so far as 130

concerns definition of my invention. I add that the steel of this composition is in certain distinguishing and characteristic feature new, and is itself the subject of a 5 separate application for Letters Patent.

The operation now described is preferably carried out in an electric furnace, and (again by way of illustration, and not limitation) I shall define in specific terms what actually 10 I use. The furnace is built with a steel shell in which is rammed a lining compounded of magnesite, some slag, and enough tar to bring it to proper consistency. The electrodes are introduced through top and bottom; those through the top (preferably there are several) extend down to the slag; those through the bottom are exposed to contact of the bath. These bottom electrodes are steel rods screwed into a copper 15 plate and tamped about with the same lining material defined above. The furnace may be stationary or tilting; the furnace which is the basis of this description is stationary, and the metal is tapped from it into 20 a ladle from which it runs into the ingot mold.

The furnace I employ has capacity sufficient to produce an ingot of about 200 pounds weight. My current is supplied at a 25 pressure of 40-45 volts. Giving again specific figures, a run of my operation continues through 6 to 7 hours; starting with a cold furnace, the consumption of current for a single run is approximately 400 kilowatt-hours. The current used may be single-phase or polyphase.

The ingot obtained in the particular run tabulated weighed 225 pounds, and in addition the test pieces aggregated 15 pounds.

40 I have said that my invention is applicable to the production of other steel alloys. That is to say, starting with iron ore or scale, and using the ferro-silicon-ferro-chromium mixture, which is the essence of 45 the invention, the desired alloy may be produced by adding (if addition be necessary), the still requisite non-ferrous ingredients—nickel, chromium, vanadium, tungsten, cobalt, molybdenum, tantalum, zirconium, or 50 what one will, in the form of oxid or of ferro-alloy.

I claim as my invention:

1. An improvement in the method of conducting the operation of smelting iron oxid 55 which consists in introducing into the charge of the smelting furnace both ferro-silicon and ferro-chromium.

2. An improvement in the method of reducing high-speed scale which consists in 60 submitting it to the smelting operation when mixed with both ferro-silicon and ferro-chromium.

3. The herein described method of producing iron alloy in continuous operation 65 from iron oxid which consists in smelting

the oxid when mingled with both ferro-silicon and ferro-chromium, and adding to the bath the desired alloying metals.

4. The herein described method of producing alloy steel in continuous operation 70 from high-speed scale which consists in smelting the scale in the presence of both ferro-silicon and ferro-chromium.

5. The herein described method of producing high-speed steel which consists in 75 smelting high-speed scale in the presence of both ferro-silicon and ferro-chromium, and in adding to the resultant bath an alloying metal of such nature as to enter in and give character to the product as a high-speed 80 steel.

6. The herein described method of producing high-speed steel which consists in smelting high-speed scale in the presence of both ferro-silicon and ferro-chromium, and 85 in adding to the resultant bath ferro-vanadium.

7. The herein described method of producing high-speed steel which consists in smelting high-speed scale in the presence of 90 both ferro-silicon and ferro-chromium, and in adding to the resultant bath a ferro-compound of an alloying metal of such nature as to enter in and give character to the product as a high-speed steel. 95

8. The herein described method of producing high-speed steel which consists in smelting high-speed scale in the presence of both ferro-silicon and ferro-chromium, together with an alloying metal, and in adding 100 to the resulting bath an alloying metal of such nature as to enter in and give character to the product as a high-speed steel.

9. The herein described method of producing high-speed steel which consists in 105 smelting in the presence of both ferro-silicon and ferro-chromium a body of high-speed scale, and subsequently building up the carbon content of the resultant bath.

10. The herein described method of producing high-speed steel which consists in smelting a mixture of high-speed scale, ferro-silicon, ferro-chromium, and carbon, the amount of carbon being insufficient to afford the desired carbon content of the 115 finished product, building up the carbon content of the resultant bath, and finally adding to the bath an alloying metal of such nature as to enter in and give character to the product as a high-speed steel. 120

11. The herein described method of producing high-speed steel which consists in smelting a mixture of high-speed scale, ferro-silicon, ferro-chromium, and carbon, the amount of carbon being insufficient to afford the desired carbon content of the finished product, and building up the carbon content in the resultant bath by introducing coke through the slag upon the bath in the furnace. 125

12. The herein described method of producing high-speed steel which consists in smelting a mixture of high-speed scale, ferro-silicon, ferro-chromium, and carbon, bringing the carbon content to a desired transient value by additions of high-speed scale, and building up thence the carbon content of the bath.
13. An improvement in the method of conducting the operation of smelting iron oxid

which consists in introducing into the charge of the smelting furnace ferro-silicon, ferro-chromium and carbon.

In testimony whereof I have hereunto set my hand.

CHARLES M. JOHNSON.

Witnesses:

BAYARD H. CHRISTY,  
FRANCIS J. TOMASSON.